

# UNITED STATES PATENT OFFICE.

FREDERICK WILLIAM GAUNTLETT, OF LONDON, ENGLAND, ASSIGNOR OF ONE-HALF TO THE SHERARDIZING SYNDICATE LIMITED, OF LONDON, ENGLAND.

## PROCESS OF DEPOSITING METALS UPON AND IN COMBINATION WITH METALS OR METAL ARTICLES.

No. 910,369.

Specification of Letters Patent.

Patented Jan. 19, 1909.

Application filed April 16, 1907. Serial No. 368,592.

*To all whom it may concern:*

Be it known that I, FREDERICK WILLIAM GAUNTLETT, of 2 Tower Royal, Cannon street, London, England, lithographic artist, 5 have invented a certain new and useful Improved Process of Depositing Metals upon and in Combination with Metals or Metal Articles, of which the following is a specification.

10 This invention relates to improvements concerning the deposition of metals in a metallic state upon, and their combination with, metals or metallic articles by the aid of applied heat, and has for its object to 15 supersede the known methods whereby for example metal such as iron in a made up form or otherwise and metal in a fine state of division such for instance as zinc dust are placed in a suitable receptacle and subjected 20 to the application of heat, for the purpose of depositing the zinc on the iron or other metal.

According to such known methods, the addition to the finely divided metal such as 25 zinc dust or a mixture of zinc and zinc oxid, or cuprous oxid or a mixture of copper and cuprous oxid, or antimony with or without some oxid of antimony before it is packed with the articles to be treated in a revolving 30 drum, for example, of a small percentage of carbon has been proposed with the object of combining with any oxygen present in the receptacle during heating, the proportion of the carbon added being 1 to 3 or 1 to 6 per 35 cent. of the amount of finely divided metal employed (see United States Patents Nos. 701,298, and 829,386, and British Patent Specifications No. 9927 of 1901, No. 28,590 of 1903 and No. 13,579 of 1904).

40 The processes thus referred to, when used for applying a deposit of zinc or analogous metal to the surface of iron or other similar metal to be coated, are known in the art as "dry galvanizing" processes. I have found 45 by experiment that these processes are capable of improvement whereby the operation is put under better control and the cost thereof is lessened. I have found that it is possible to form an alloy between the coating 50 metal and the metallic surface of the object to be coated without necessarily maintaining all portions of the metallic surface to be coated in actual contact with the coating material.

In practicing this invention the finely divided metal to be deposited (hereinafter for convenience called the coating metal) is mixed with a substantial amount equal to and preferably exceeding that of the coating metal of a substance (not being an oxid of the coating metal) which is chemically inert with respect to the coating metal at the temperature necessary for the deposition or decremental combination of the coating metal with the metal or metallic article to be coated.

As examples of substances which answer the requirements of being chemically inert under the conditions specified, carbon and silica in various degrees of fineness may be 70 cited, and these substances it may be observed remain chemically inert with respect to the finely divided coating metal, e. g. zinc dust say below a temperature of 1500° F., while I find from experiments that the finely 75 divided coating metal, e. g. zinc dust will combine with the metal or metallic articles at a temperature considerably below that mentioned above.

It may here be observed that the presence 80 of some oxid of the metal is not adverse to the process; the temperature being such that the carbon material employed will not effect the reduction of the oxids of the metals.

The proportions of the inert substance and 85 the metal in a fine state of division I have found may vary very considerably according to the particular result required to be obtained, but by way of example only, a somewhat general proportion may be taken as being 90 nine parts by volume or thereabouts of the chemically inert substance to one part or thereabouts of the finely divided metal or metals.

In effecting the combination of the finely 95 divided coating metal with the metal in made up form or otherwise the latter is enclosed with the mixture in a suitable receptacle and subjected to heat, as by placing the receptacle in a gas or otherwise heated oven. 100

Taking as a typical example, the coating of iron or steel with zinc by employing in the manner indicated a mixture of nine parts by volume of sand and one part by volume of zinc dust, the receptacle in which the metal 105 or metallic articles and the mixture are placed is heated up to a temperature of about 700° F. for about one hour. The duration

and temperature of heating is however even in this example very considerably variable according, for instance, to the dimensions of the receptacle and the depth of coating required.

By the process according to this invention the results secured generally, and those particularly pertaining to the cost of effecting the combination of the finely divided coating metal with, and its deposit on metal or metallic articles and the qualities and properties of the articles treated according to the process constitute an important advance in the art. The results obtained may be also greatly varied according to (a) the fineness or coarseness of the inert substance, (b) the time of treatment, (c) the heat to which the articles and mixture are subjected and (d) the variation in the proportion of the inert substance to the coating metal. In this latter connection I may observe that, other things being equal, as the proportion of the coating metal to the inert substance is reduced the greater it is believed is the alloy between the divided coating metal and the metal or metallic articles.

It is impossible to state the exact conditions necessary to meet each particular case as the exact conditions vary with the metals employed and the proportions of the inert material and the results required but in each case the working conditions for effecting the object desired can be ascertained by one or two trial experiments.

What I claim and desire to secure by Letters Patent is:—

1. The process of depositing metals upon metals, which process consists in applying to the metal to be coated a mixture of the

coating metal or metallic compound in finely divided form, and a large quantity of a substance, not being an oxid of the coating metal, which is chemically inert to the coating material at the temperatures necessary for depositing the metallic coating upon, and in combination with the foundation metal, and submitting the whole to heat, the inert substance being present in a quantity equal to and preferably in excess of that of the coating material, substantially as described.

2. The process of depositing zinc upon iron, steel or other metal, which process consists in applying to the metal to be coated zinc dust or finely divided zinc mixed with a substance, not being an oxid of the coating metal, which is inert to the zinc dust or finely divided zinc at the temperature necessary for depositing the metallic coating upon and in decremental combination with the foundation metal, and submitting the whole to heat, the inert substance being present in a quantity at least equal to that of the coating metal, substantially as described.

3. The process of depositing metals upon metals, which process consists in applying to the metal to be coated a mixture of the finely divided coating metal or metallic compound and sand or other form of silica or like material in quantity at least equal to said coating metal or compound, and submitting the whole to heat, substantially as described.

In witness whereof I have hereunto signed my name in the presence of two subscribing witnesses.

FREDERICK WILLIAM GAUNLETT.

Witnesses:

ROBERT MILTON SPEARPOINT,  
H. D. JAMESON.